

Aug. 12, 1952

R. A. NEISH

2,606,866

METHOD OF TREATING TIN PLATE

Filed Oct. 27, 1948



*Inventor:*  
RICHARD A. NEISH,  
*by:* Donald G. Dalton  
*his Attorney.*

Patented Aug. 12, 1952

2,606,866

# UNITED STATES PATENT OFFICE

2,606,866

## METHOD OF TREATING TIN PLATE

Richard A. Neish, Pittsburgh, Pa., assignor to  
United States Steel Company, a corporation of  
New Jersey

Application October 27, 1948, Serial No. 56,843

2 Claims. (Cl. 204—56)

1

This invention relates to an improved method of treating tin-plate such as that used in making cans. The object of the invention is to produce tin-plate which is resistant to the formation of yellow stain during storage, to discoloration such as occurs during the heat curing of enamels, to etching, and to sulfide staining such as customarily occurs in the can, and is adapted, furthermore, to serve as a suitable base for subsequent lacquering.

Numerous methods have been proposed for treating tin-plate to improve its characteristics and inhibit the development of defects such as baking discoloration and sulphide stain which usually show up only after the material has been used for its ultimate purpose such as lithographing stock or containers for food. Some of these methods have been successful in a measure but none of them has provided a complete solution of the problem. Stevenson Patent No. 2,424,718, for example, discloses a method which increases resistance to sulphide discoloration but does not prevent baking discoloration. It is accordingly a further object of my invention to provide a method superior to those previously suggested, in effectiveness, speed, and economy.

Yellow stain on tin-plate is known to be the visible manifestation of atmospheric oxidation of the exposed surface of the tin. Both chemical and electrical oxidation (by anodizing) have been recommended as means for minimizing this defect. Neither one is sufficiently effective alone, however, to prevent this discoloration, although a dense coating of anodic oxide gives some protection and increases resistance to sulphide staining. Another prior method of treating tin-plate makes use of the fact that tin oxides form complex compounds with many passivating radicals (chromates, phosphates, molybdates, etc.) which provide a surface layer inhibiting to a degree, further oxidation as well as chemical attack by dilute acids or alkalies. The difficulty is that such a treatment converts only the outer surface of the original oxide, and the surface portion so affected is extremely thin and comparatively permeable so that the cushion of unconverted oxide beneath the superficial protective layer can continue to grow and eventually results in the appearance of yellow stain. Similarly and for the same reasons, this superficial protective layer does not offer comparable resistance to sulfide staining or to chemical attack, and is found to be less resistant to mechanical abrasion arising from operation of the treating and related processes. Even though cathodic electrolytic clean-

2

ing be resorted to before such an immersion treatment, the oxide reforms on the tin surface immediately the cathodic action ceases, and the net result is again a cushion of unconverted oxide beneath a thin superficial protective layer.

I have discovered a method of treating tin-plate whereby the initial oxide coating resulting from atmospheric oxidation is reduced in the presence of a passivating radical. This insures 10 that re-oxidation will occur under conditions causing the formation of an effective protective film of the desired complex directly on the tin without an intermediate layer of oxide. Generally speaking, my method involves the cathodic 15 cleaning of tin-plate in an electrolyte including passivating radicals, followed immediately by anodizing the material in the same electrolyte. This causes reduction of the oxide film initially present on the material and permits the film of 20 the complex to be then built up quickly to a thickness sufficient to inhibit subsequent oxidation of the tin therebelow. After extensive experiment, I have found that chromates or mixed 25 chromates and phosphates are most desirable as passivating radicals, all things considered.

More particularly, my invention consists in passing tin-plate through a dilute solution containing chromate ions or a mixture of chromate and phosphate ions and making the material first 30 a cathode and then an anode. As a result, the oxide film initially present on the material is first reduced and then reformed in the presence of passivating radicals with which the oxide combines to form complex polymolecular groups constituting a water-insoluble, dense, adherent and 35 continuous film affording protection against further oxidation and chemical attack. Further, the amount of complex protective film so formed is controllable by means of the anodic current density and the time interval allowed. Good results are 40 obtained from a solution containing from .2 to 2% of a chromate, e. g., the chromate of an alkali metal such as sodium dichromate

( $\text{Na}_2\text{Cr}_2\text{O}_7 \cdot 2\text{H}_2\text{O}$ )

45 While the total salt concentration may be varied considerably, decreasing it below 1.5% reduces the conductivity substantially and concentrations less than .2% are relatively ineffective. Conversely, increasing the concentration above 2.0% does not result in a significant improvement although slightly higher concentrations, say 3.0%, may be commercially advisable for the purpose of increasing the time interval before replenishment is necessary. Instead of the dichromate

alone, I may use a mixture thereof with a phosphate of an alkali metal such as sodium di-hydrogen phosphate ( $\text{NaH}_2\text{PO}_4 \cdot 2\text{H}_2\text{O}$ ). The ratio of phosphate to dichromate may be about 1:1, e. g., .8% of each, or the phosphate may be used in a larger amount such as 1.5% phosphate with .2% dichromate.

The solution is normally acid and is preferably maintained at an acidity corresponding to a pH value between 7 and 4 by adding sulphuric acid, if necessary. I have produced resistant films at various acidities between pH 2 and 11; however, a pH less than 4 does not improve results, while films formed at a pH greater than 7 do not offer satisfactory adherence with certain types of tin-plate lacquers.

The action of the treatment in forming a protective film appears to be independent of temperature at least in the range between room temperature and 180° F.

The method of my invention may be carried out most efficiently by drawing a continuous strip of tin-plate, such as that produced by known electrolytic tinning processes, through the solution described above and past electrodes immersed therein with respect to which the strip is first made a cathode and then an anode. The process may be conveniently practiced by the aid of apparatus shown diagrammatically in the single figure of the accompanying drawing.

Referring in detail to the drawing, tinned steel strip is unwound from a coil 10 and passed through a bath of the aforesaid solution contained in a tank 11 provided with entry and exit guide rollers 12 and 13 and hold-down rollers 14. Spaced pairs of electrodes 15 and 16 are immersed in the bath, the electrodes of each pair being on opposite sides of the path of the strip. A current source such as a generator 17 is so connected to the strip and electrodes 15 as to make the portion of the strip between them the cathode. A similar source 18 is so connected to the strip and electrodes 16 as to make the portion of the strip between them the anode. Connections to the strip are shown as made through rollers 12 and 13 which must therefore be conducting and insulated from the tank if it is also conducting but any other suitable form of connection to the strip may be used. After emerging from the solution in tank 11, the strip passes through rinsing and drying apparatus indicated at 19 and 20, respectively, and is then wound up by a recoiler 21 which exerts the tension necessary to pull the strip through the line of processing apparatus.

The strip may be processed at speeds of several hundred feet per minute, since the treatment requires only a very short time. Operating at 450 feet per minute, for example, with electrode 5' long, gives good results although the time of exposure of a given point on the strip to cathodizing is only .6 or .7 second and the same for anodizing. The current density required for the cathode treatment will vary with the degree of initial oxidation of tin surface, and with the allowable time interval, but 100 amperes per square foot is about the maximum needed, while a much lower density, such as 30 amperes, has been found satisfactory in some instances. The thickness and characteristics of the films obtained will depend upon the anodizing process; that is, they are a function of the time and the current density. I have produced films by using anodic current densities ranging from one to 90 amperes per square foot. However, those formed with a current density greater than 30 amperes per square

foot tend to be more porous in nature, are less protective, and are not generally suitable as lacquer bases. Film produced with an anodic current density of 10 to 30 amperes per square foot are protective and suitable for certain applications, although the adherence of phenolic type lacquers may be poor. The most effective films for all purposes, however, are produced with a current density of 1 to 10 amperes and more specifically 4 to 7 amperes.

Tin-plate processed according to my invention exhibits improved characteristics in several respects, in comparison with material treated by methods known previously. In the first place, it has less tendency to discoloration and sulphide staining as well as good resistance to etching in dilute acid. It is further characterized by good adherence of phenolic tin-plate lacquer. This adherence is better, the lighter the layer of protective film laid down during the anodic treatment. The product of my method also shows better solder-flow characteristics as measured by capillary rise. Furthermore, the adhesional strength of the soldered areas is not adversely affected.

Most oxide films have little resistance to abrasion, but material treated according to my invention acquires an oxide coating having greater resistance than the products of known methods. In fact, the protective film produced by my method is comparatively unaffected by abrasion on passing through the apparatus comprising the processing line.

My improved method produces a uniform protective film which may be easily controlled as to thickness. Use of the phosphate radical produces a surface of pleasing appearance which is non-toxic, tasteless and odorless. The process may be carried on at high speed in a continuous production line, since the film formation requires only a second or less with suitable current density. The cost is low because of the high speed which is practical and the cheapness of the salts employed. There is no factor in the control of the method which is unduly critical. The process utilizes the electrical resistance of the protective film to insure uniform and complete coverage. That is to say, when the film has been formed on a given area of the tin-plate, no further oxidation occurs therein because of the electrical resistance of the film, until all other portions of the material in the bath have been coated to the same thickness. The rate of film formation is a maximum at the beginning thus insuring immediate protection at all points on the surface of the material.

While the specific example of the method described in detail hereinabove involves the processing of tinned strip, the invention is also applicable to the treatment of tinned sheets such as produced by the hot-dip method of coating tin-plate.

Although I have described only a preferred practice of the invention with certain modifications, it will be understood that changes in the procedure disclosed may be made without departing from the spirit of the invention or the scope of the appended claims.

I claim:

1. In a method of treating sheet material having a tin surface, to inhibit the tendency thereof to sulphide staining and baking discoloration and increase the adherence of lacquer, the steps including first making the material cathode in an acid solution containing from .2 to 3% of a

chromate of an alkali metal and having a pH value of from 2 to 7, thereby at least partially reducing the oxide film initially existing on the material, and immediately thereafter making the material anode while still in said solution, thereby re-oxidizing the tin surface and forming thereon a water-insoluble protective film of a complex combination of the oxide and said chromate.

2. The method defined by claim 1 characterized by said solution containing an alkali-metal phosphate and a chromate aggregating about 3.0% or less.

RICHARD A. NEISH.

REFERENCES CITED

The following references are of record in the file of this patent:

UNITED STATES PATENTS

| Number      | Name        | Date           |
|-------------|-------------|----------------|
| 2,215,165   | Sumner      | Sept. 17, 1940 |
| 2,312,076   | Cook et al. | Feb. 23, 1943  |
| 5 2,424,718 | Stevenson   | July 29, 1947  |
| 2,450,509   | Glock       | Oct. 5, 1948   |
| 2,503,217   | Frust       | Apr. 4, 1950   |

FOREIGN PATENTS

| 10 Number | Country       | Date          |
|-----------|---------------|---------------|
| 416,608   | Great Britain | Mar. 21, 1934 |
| 486,752   | Great Britain | June 9, 1930  |